

W. P. DREAPER.

MANUFACTURE OF ARTIFICIAL FILAMENTS AND THE LIKE.

APPLICATION FILED JAN. 16, 1922.

1,437,341.

Patented Nov. 28, 1922.

2 SHEETS—SHEET 1.

Fig. 1.



INVENTOR  
William P. Dreaper

By  
James L. Dorn,  
Attorney.

W. P. DREAPER.

MANUFACTURE OF ARTIFICIAL FILAMENTS AND THE LIKE.

APPLICATION FILED JAN. 16, 1922.

1,437,341.

Patented Nov. 28, 1922.

2 SHEETS—SHEET 2.



Fig. 2.



INVENTOR  
William P. Dreaper

By  
Howard L. Morris  
Attorney

## UNITED STATES PATENT OFFICE.

WILLIAM PORTER DREAPER, OF LONDON, ENGLAND.

## MANUFACTURE OF ARTIFICIAL FILAMENTS AND THE LIKE.

Application filed January 16, 1922. Serial No. 529,735.

*To all whom it may concern:*

Be it known that I, WILLIAM PORTER DREAPER, a subject of the King of Great Britain, residing at London, England, have 5 invented new and useful Improvements in the Manufacture of Artificial Filaments and the like, of which the following is a specification.

The manufacture of staple fibre by cutting artificial silk skeins into short lengths of say four inches and using this for the production of spun yarn has naturally followed the process of manufacture of artificial silk up to the time where the skeins 10 are finally cut up as described. On cutting, the short lengths of filament gradually separate as the short lengths of strand gradually loose their twist or throw. The staple fibre here referred to is a bright and silk 15 like product similar in appearance to artificial silk except that it is present as filaments of predetermined length.

In the present invention the process of manufacture is materially simplified and 20 the production of a twisted yarn similar to that of artificial silk is obviated, but at the same time filaments in staple fibre form are finally obtained possessing the brightness and softness of ordinary artificial silk. 25 Also it is possible to produce staple fibre of this quality in increased quantity over that ordinarily obtained when such staple fibre is prepared from inferior or rejected skeins of artificial silk prepared originally 30 in ordinary sizes.

According to my invention, the strands of filaments as they leave the spinning bath are led directly on to the arms of a suitable winder to be hereinafter described, distributing the strands on the same in the 35 manner to be described. In this way an ordered skein of filaments arranged in parallel form is obtained which could not be ordinarily rewound in strand form as it 40 comes from the composite jets as in the case of artificial silk. These filaments can then be subsequently treated in any way that is required without damage and ultimately dried in a stretched condition either on the 45 original winder or after removal from the same on a stretching frame. Thus by immediately forming the issuing filaments into skeins, and cross-lacing the skeins, they 50 can be handled with facility and they are 55 in a state of order in which they remain until the skeins are finally cut up so as to

obtain filaments of predetermined lengths, which completes the production of staple fibre which has the qualities of ordinary artificial silk so far as evenness of filament 60 and brightness and softness are concerned.

A suitable apparatus for carrying the said invention into practice is shown in the accompanying drawings in which:—

Figure 1 is a side elevation and 65

Figure 2 a vertical central section.

The strand A of filaments possibly to a number of 200, (e. g. produced from a single jet which contains the requisite number of holes) are led down the precipitating 70 bath and then out of the same over a suitable guider-wheel B which is adapted to rotate and also move axially on a shaft C. The guider is reciprocated axially on the shaft C by means of a roller D which rolls 75 in an annular groove E in the hub of the guider and has a reciprocatory motion imparted to it in any known manner through the rod F. In some cases the wheel B may be replaced by a reciprocating guide fork 80 of glass or other suitable material. By this means the strand of filaments A is spread on the working surface of the arms of a skein winding frame or winder, which is of such a diameter that a full sized skein is 85 at once produced at this early stage of manufacture, in which form it remains until the filaments are finally cut up into short lengths and become staple fibre. The skein winding frame, comprises a series of 90 arms G, G' mounted on a hub H secured to a driving shaft J, that turns in bearings K, K and is provided with a driving pulley L. Four of the arms G, G are made rigid and have segmental flanged ends M, M to 95 receive the strand. The remaining two diametrically opposite arms G', G' are made in two relatively movable parts, their outer parts N, N being made separately and adapted to slide in guideways O, O in the 100 outer ends of the fixed inner parts G', G'. The outer parts N, N bear the flanged ends M, M and are slotted at P, P to receive screw-threaded studs Q, Q fixed on the arms G', G' and provided with fly-nuts R, R to 105 enable the movable parts N, N to be secured in any positions to which they may be adjusted. The exact positions to which the parts N, N are set may be determined by means of distance-pieces S, S arranged between the inner ends of the parts N, N and the hub H, one pair of distance-pieces be- 110

ing used when the strand is being wound on the frame and another thicker pair when the wound skein is to be stretched. The parts N, N may also be provided with 5 graduations, as indicated at T in Figure 1, to facilitate adjustment to any desired position. If desired more or all of the arms may be made adjustable as above described.

The apparatus above described is only 10 given by way of example.

In an alternative form the guider may remain stationary and the winder G, M may move from side to side so that the same 15 effect is produced.

15 The strands wound to such a suitable diameter and the filaments openly packed by the side to side movement of the said guider B are subsequently washed or otherwise treated on the winder G, M and with advantage 20 also finally dried on the same in a stretched condition, so that the required brightness of the staple fibre can be obtained. The filaments are thus produced in quantity and at a cheaper rate than they 25 could otherwise be produced. All handling of the filaments is obviated, also any loss through rewinding such as occurs in ordinary artificial silk production. The winders may be long enough to hold several such 30 skeins of filaments as these are wound side by side on the arms of the winder from a corresponding number of jets in the bath, separate guiders being preferably employed.

35 The removal of the surplus water from the skein just before the process of drying in a stretched condition may be facilitated by rapidly revolving the winder so as to throw off the surplus water by centrifugal force. The drying may be assisted by directing 40 a strong blast of air on to the surface of the skein whilst the latter is revolved as above mentioned.

When sufficient strand has been collected on the winder the skein so formed is cross 45 laced in, for example, three equidistant places, to prevent any slipping or disarranging of the filaments and at this stage the skein may be removed from the winder by shortening one or more of these arms and 50 handled from this stage, as a skein of artificial silk might be, and finally dried in the required stretched condition to ensure brightness.

55 Preferably however the skein is kept on the winder and washed or otherwise treated on the same. To effect this the winder may be removed from its position and mounted over a bath of water or other liquid or a succession of baths in such a manner that 60 it revolves and dips at its lower part into the said solution and is thus treated evenly with the same solution or solutions. When it is required to dry the skein of filaments in a stretched condition on the original 65 winder, one or more of the said arms over

which the filaments have been wound are by suitable means extended just before drying so that the required stretch is given to the filaments.

If for any reason it is desired to start the 70 washing or treating operations directly the filaments are wound this can be effected by allowing the revolving winder to just dip into a bath of the required liquid.

If it is desired to introduce a small percentage 75 of natural silk, this can be effected by winding on to the winder, at the same time as the filaments are wound, a single thread of silk which will give the required admixture. In this case it is possible to 80 degum the silk used if this is raw silk by some suitable treatment before the skein is cut up into short lengths. For instance if a 20-denier silk thread is so wound with the artificial filaments and if the latter will 85 give a 600 denier thread or strand in the dry, the proportion of natural silk to the artificial filaments will be indicated, i. e., 1 to 30. The admixture of natural and artificial silk will then be complete, but care 90 must be taken not to stretch the skein in the final drying operation to such an extent that either the natural silk is damaged or that the natural silk cuts through or damages the artificial filaments.

If the filaments are to be dyed before they 95 are cut up into staple fibre this may still be done on the winder if provision is made for the arms to be suitably relaxed during the time of dyeing.

100 What I claim is:—

1. A process of producing staple fibre, consisting in that a strand of artificial silk is wound in an untwisted condition on to a skein winding frame, treated with a suitable 105 liquid, stretched, dried in such stretched condition, and then cut up into suitable lengths for forming staple fibre.

2. A process of producing staple fibre, consisting in that a strand of artificial silk 110 is wound in an untwisted condition on to a skein winding frame, treated with a suitable liquid on such frame, stretched by forcibly expanding such frame, dried in the stretched condition, and then cut up into suitable 115 lengths for forming staple fibre.

3. A process of producing staple fibre, consisting in that a strand of artificial silk is wound in an untwisted condition on to a skein winding frame, treated with a suitable 120 liquid on such frame, subjected to centrifugal force by rapidly revolving the frame, stretched by forcibly expanding the frame, dried in the stretched condition, and then cut up into suitable lengths for forming 125 staple fibre.

4. A process of producing staple fibre, consisting in that a strand of artificial silk is wound in an untwisted condition on to a skein winding frame, the skein is cross 130

laced, treated with a suitable liquid, stretched, dried in such stretched condition, and then cut up into suitable lengths for forming staple fibre.

5 5. A process of producing staple fibre, consisting in that a strand of artificial silk is wound in an untwisted condition on to a skein winding frame in conjunction with natural filaments, treated with a suitable 10 liquid, stretched, dried in such stretched condition, and then cut up into suitable lengths for forming staple fibre.

6. A process of producing staple fibre having the lustre of the artificial strand, from 15 strands of artificial silk, consisting in winding a strand of artificial silk in untwisted condition, treating the filament so wound with a suitable liquid, subjecting said filament to stretching force outwardly in a plurality of opposite radial directions, subjecting the filament to centrifugal force and to 20 a blast of air, drying in the stretched condition and cutting into lengths to form a staple fibre.

25 7. A process for producing staple fibre from strands of artificial silk and retaining the lustre of the strands, consisting in wind-

ing a strand of artificial silk in an untwisted condition on to a skein winding frame, treating it with a suitable liquid while on the 30 frame, stretching it by forcibly expanding the frame in a plurality of opposite directions, drying it in the stretched condition on the frame, treating it with a liquid and relaxing the tension of the frame during 35 said treatment, drying the strands and cutting them into staple lengths.

8. A process for producing staple fibre from strands of artificial silk and having the lustre of said strands, consisting in winding a strand of artificial silk in an untwisted condition on to a skein winding frame, treating it with a suitable liquid while on the frame, stretching it by forcibly extending said frame, treating it with a dye liquid, the 40 tension due to the frame being relaxed during such treatment, drying the strand and cutting into suitable lengths for forming 45 staple fibre.

WILLIAM PORTER DREAPER.

Witnesses:

CONRAD ARNOLD,  
WALTER ROBINSON.